

Nov. 1, 1938.

E. R. BOLLER

2,135,030

TREATMENT OF WOOD

Filed July 19, 1935



INVENTOR.

ERNEST D. BOLLER.

BY

Albert B. Briggs.

ATTORNEY.

## UNITED STATES PATENT OFFICE

2,135,030

## TREATMENT OF WOOD

Ernest R. Boller, Cleveland Heights, Ohio, assignor, by mesne assignments, to E. I. du Pont de Nemours & Company, Wilmington, Del., a corporation of Delaware

Application July 19, 1935, Serial No. 32,162

9 Claims. (Cl. 21—35)

This invention relates to processes for depositing preservative compositions, fireproofing compositions, and the like, within a porous material, and is particularly directed to such processes wherein such impregnating agents are carried into the porous materials in dimethyl ether.

It is now the customary practice to preserve wood by submerging it in a water solution of a preserving salt, such as zinc chloride, and then injecting the solution into the wood by the use of pressure. After a desired degree of penetration of the wood has been effected, the aqueous solution is ordinarily allowed to drain from the pressure receptacle. Water which is retained in the wood must subsequently be removed by kiln drying or air seasoning.

The injection of water into the wood causes considerable swelling and, upon drying, the consequent shrinkage of the wood is attended by a certain amount of warping, checking, and raising of the grain. The extent of this deterioration of the wood depends largely, of course, upon the characteristics of the wood being treated and, to a lesser degree, upon the care exercised in the treating and drying procedures. When the treated wood is to be employed in certain relations, this deterioration is not particularly disadvantageous, but wood which is warped and checked cannot satisfactorily be used for a large number of purposes.

Aqueous vehicles are further unsatisfactory because of the relatively long time and the high pressures required to effect a satisfactory impregnation of wood. Moreover, the large amount of time required to dry the wood after its impregnation with an aqueous menstruum results in high equipment and operating costs if it is kiln dried, and in high carrying charges if it is air seasoned.

The customary processes of impregnating wood by means of an aqueous vehicle have also been found disadvantageous by reason of the relatively large and expensive equipment required for the ordinary pressure processes. In addition to the expense attendant upon the installation and maintenance of such equipment, there is the additional disadvantage that the equipment is not readily adaptable to various types of wood which require modified methods of treatment.

Aqueous vehicles offer yet another disadvantage in that a large number of impregnating agents are not water soluble and cannot, therefore, be used in water solution.

Considered together, the above enumerated disadvantages have prevented the impregnation of wood by the use of an aqueous menstruum in

many commercial applications. It has been impractical to impregnate finished or semi-finished lumber with suitable agents for staining, fireproofing, or preserving the wood.

It has been proposed to avoid the difficulties encountered when wood and the like are impregnated by the use of aqueous vehicles, by using non-aqueous menstrua. It has, for instance, been suggested that alcohol, or liquid hydrocarbons such as gasoline or kerosene be used. Such non-aqueous vehicles display the same disadvantages as do aqueous vehicles, to a greater or lesser extent, and they have the further disadvantage of being quite expensive. In addition to the fact that the non-aqueous solvents heretofore employed are high in cost for an initial installation, their expense is rendered even greater by the fact that it is almost impossible to recover the solvent from the porous material.

When wood is to be impregnated with a preservative salt, such as zinc chloride, if a non-aqueous menstruum is to be employed, it has been proposed to use alcoholic solutions of zinc chloride. Alcohol causes warping and checking of wood, though to a somewhat smaller extent than does water. Alcohol, moreover, causes a raising of the grain of the wood, and, accordingly, like water, is unsuitable for treating finished wood.

After such a non-aqueous menstruum has been injected into wood, either by pressure processes or by simple immersion, it is impractical to attempt recovery of the menstruum. It is, of course, theoretically possible to recover such non-aqueous menstrua, but the cost of such operations would be prohibitive. In a pressure process of impregnation, there is, of course, a certain amount of heat in the wood, but this heat is inadequate to distill off the relatively high-boiling menstruum heretofore used. The poor heat conduction of wood, moreover, makes it impractical to distill off the vehicles by the application of heat from an external source. It is the ordinary practice to recover only the portion of the non-aqueous vehicle which can be drained from the wood, and no attempt is made to recover the fluid retained in the wood.

Processes employing non-aqueous menstrua for the pressure impregnation of wood require equipment comparable in size and cost to that used in processes employing aqueous vehicles. Processes employing non-aqueous menstrua also require relatively long periods of time for the impregnating and drying operations.

It is an object of my invention to provide proc-

esses which can be employed for the impregnation of wood and the like without damage thereto. It is a further object of my invention to provide processes whereby wood may be impregnated with desired impregnating agents without the deleterious swelling, shrinking, warping, checking, and raising of the grain which attends the use of most of the menstruums hitherto known. A still further object of my invention is to provide processes whereby finished lumber may satisfactorily be impregnated with suitable fireproofing, staining, and preservative agents. A still further object of my invention is to provide processes whereby a deep and uniform penetration of impregnating agents can quickly and economically be achieved. A still further object of my invention is to provide processes which are low in cost, and which can readily be adapted to the condition of the wood. Other objects of my invention will become apparent hereinafter.

My objects are accomplished, briefly, by impregnating wood or the like with suitable impregnating agents carried in dimethyl ether. The dimethyl ether may, of course, be diluted with less expensive, low boiling materials such as carbon dioxide.

Wood and the like may be impregnated according to the processes of my invention with impregnating agents such as pigments, lakes, dyes, stains, resins, gums, lacs, oils, waxes, parasiticides, and fireproofing compositions. Many water insoluble impregnating agents can be dissolved in dimethyl ether, and it is thus possible to use such water insoluble impregnating agents in an economical and practical manner. For instance, such preservatives as beta-naphthol, tetrachlorophenol, and orthophenylphenol may be used in dimethyl ether. I may also use mixtures of various impregnating agents.

Dimethyl ether is a solvent for a wide variety of impregnating agents, but there may be found an impregnating agent which is not soluble therein. In such an instance, some of the advantages of my invention may be obtained by dispersing the impregnating agent in the menstruum, but it is usually desirable to employ impregnating agents which are soluble in the dimethyl ether.

The impregnation of wood or the like may be accomplished by simply immersing it in the dimethyl ether solution. However, it is usually preferred to inject the non-aqueous vehicle into the wood by the use of pressure. Pressures up to the critical pressures of the dimethyl ether may be obtained by heating it. Because of the low boiling point of dimethyl ether, no large amount of heat will be required to obtain relatively high pressures, and, under many circumstances, satisfactorily high pressures may be obtained without the addition of external heat by reason of the normal pressure of the dimethyl ether at ordinary temperatures.

Dimethyl ether is characterized by its relatively low surface tension and its relatively low viscosity. The impregnation of wood according to the processes of my invention, accordingly, proceeds very rapidly even at rather moderate pressures, a satisfactory degree of penetration being obtained in a relatively short period of time. This, of course, is very important from an economic standpoint because smaller equipment may be used for handling a given amount of lumber.

After a desired degree of penetration has been obtained, the dimethyl ether is drained from the wood. After the liquid has been drained off, the liquid remaining in the wood can readily be re-

moved therefrom by permitting it to boil off. Ordinarily, no addition of heat is necessary to effect an almost complete evaporation of the dimethyl ether, but, if desired, additional heat may be supplied. The gas which results from the boiling of the dimethyl ether can be recovered and condensed, whereupon it may be used as a solvent for more of the impregnating agent.

It will be apparent that the removal of dimethyl ether is exceedingly easy of accomplishment, and it is to be noted that a substantially complete recovery of the dimethyl ether is practical. The short time required to effect a separation of the liquid from the wood is, of course, highly advantageous.

In order that the preferred sequence of steps in a specific process for the impregnation of wood may be better understood, there is illustrated in the accompanying drawing a flow sheet of such a typical process.

Wood to be impregnated is placed in the treating cylinder, and a solution of a suitable impregnating agent, for instance zinc chloride, in dimethyl ether is admitted to the treating cylinder from the solution storage tank. The wood to be impregnated is placed in the treating cylinder and subjected to a vacuum, by means of the indicated vacuum pump, to remove most of the air from the cylinder and the wood. The cylinder is then connected to the solution storage tank, which is at a higher temperature than the cylinder, and the solution of impregnating agent flows into the cylinder under its own pressure.

The desired temperatures and the corresponding pressures are maintained in the treating cylinder by the use of steam coils. The desired temperature and pressure are maintained for the time required to effect the desired degree of penetration of the wood. At the end of this time, the line between the treating cylinder and the solution storage tank is opened, and the solution is forced from the treating cylinder into the solution storage tank which at this time, of course, is at a lower temperature and pressure than the treating cylinder.

After the solution has been drained from the wood and forced into the solution storage tank, the line between the cylinder and the solution storage tank is closed, and the line from the treating cylinder to the condenser is opened. The dimethyl ether which has been retained in the wood distills therefrom and is condensed in the condenser from which it is led to a receiving tank. The temperature of the wood is ordinarily sufficient to supply the heat required to vaporize substantially all of the menstruum.

The atmosphere of the vaporized dimethyl ether which remains in the treating cylinder is finally swept out with air from a blower, and dissolved in a suitable solvent, such as 60° Bé. sulfuric acid, in a scrubber. From time to time the dimethyl ether which has been dissolved in the scrubber is removed from the solvent liquid by heating, and the vaporized dimethyl ether is returned through the condenser to the receiving tank and then to the solution storage tank.

The condensed liquid in the receiving tank is heated somewhat and forced, under its own pressure, through the dissolver where a desired amount of the impregnating agent is put into solution. It will be noted that a suitable storage tank for the liquid is provided, which storage tank is equipped with heating and cooling means whereby the pressure may be adjusted.

After the dimethyl ether has been evaporated

from the wood, and after any remaining gases have been swept from the cylinder by means of the blower, the wood, which is now entirely dry, can be removed from the cylinder. The wood is then ready for use, and no further seasoning or drying is required.

Considering my invention with more particular reference to certain illustrative impregnating agents and certain dimethyl ether solutions, the following examples are given:

*Example I*

Following the procedure above outlined, a number of samples of finished wood were subjected to a 5% solution of zinc chloride in dimethyl ether. Temperatures of from 40 to 50° C. were maintained with corresponding pressures from 130 to 150 pounds per square inch. These conditions were maintained for 30 minutes. The woods thus treated were as follows: California white pine, heart and sap, 1½" x 2" x 4"; Wisconsin white pine, sap, ¾" x 2" x 4"; Douglas fir, heart, 1¼" x 1¼" x 4"; red oak, heart, ¾" x 4" x 4". All of these specimens treated according to the procedure of this example were completely impregnated with zinc chloride. There was no discernible swelling, warping, or raising of the grain of these finished pieces of wood.

*Example II*

A cylinder of seasoned heart white oak, 3½" in diameter and 4" long, was subjected to a 5% solution of zinc chloride in dimethyl ether for three hours at temperatures of 40 to 50° C., and at corresponding pressures of 130 to 150 pounds per square inch. The wood used in this example is practically impenetrable by aqueous solutions, but under the conditions of this example, approximately half of the wood was impregnated with zinc chloride. There was no apparent swelling, checking, or distortion of the wood.

*Example III*

Following the procedure of the above examples, a number of pieces of Ponderosa pine window sash were treated with a 5% solution of zinc chloride in dimethyl ether. The treatment was conducted at 150 pounds per square inch pressure for thirty minutes for sapwood and forty-five minutes for heartwood. There was no perceptible swelling, warping, checking, or roughening of the surfaces of the wood. Examination of typical specimens showed complete penetration of the wood with zinc chloride, and about one pound of zinc chloride was retained per cubic foot.

*Example IV*

Following the procedure of Example III, but using dimethyl ether containing dissolved there-in about twenty per cent of carbon dioxide as the solvent for zinc chloride, a number of pieces of finished lumber were impregnated. Excellent results were obtained, and it is noted that a somewhat more rapid penetration of the wood seemed to be obtained than when the dimethyl ether was used alone as a solvent.

It will be readily understood that numerous modifications may be made in the above illustrative examples without departing from the spirit of my invention. The impregnating agent used and its concentration will depend, of course, upon the characteristics which it is desired to impart to the wood.

The pressures of treatment may also be widely varied and they will be determined for each case

by the penetration desired, the nature of the wood, the temperature of treatment, and the length of treatment. When materials which can easily be impregnated are treated, it is, of course, unnecessary to use such high pressures, and the processes of my invention may, under some circumstances, advantageously be practiced at atmospheric pressures or at pressures only slightly above atmospheric.

It will also be understood that the scheme of operation illustrated in the accompanying drawing may be widely varied without departing from the spirit of my invention. Instead of condensing the vaporized dimethyl ether by means of refrigeration, the gas may be condensed by the use of a compressor. It will be readily apparent, moreover, that the processes already known for the impregnation of porous materials by the use of aqueous menstruums and by the use of high boiling non-aqueous menstruums may readily be adapted, according to the teachings of my invention, to the use of dimethyl ether.

While I have shown certain specific impregnating agents, certain dimethyl ether solutions and certain procedures and conditions of operation, it will be understood that I do not intend to be restricted thereby, the scope of my invention being apparent from the following claims:

I claim:

1. In a process for the impregnation of a porous material, the step comprising immersing the material in a liquid, non-aqueous menstruum comprising dimethyl ether, the menstruum carrying an impregnating agent. 35
2. In a process for the impregnation of wood, the step comprising immersing the wood in a liquid, non-aqueous menstruum comprising dimethyl ether, an impregnating agent being dissolved in the menstruum. 40
3. In a process for the impregnation of wood, the steps comprising immersing the material in a liquid, non-aqueous menstruum comprising dimethyl ether, the menstruum having an impregnating agent dissolved therein, and, after 45 impregnation of the wood, recovering the portion of the menstruum retained therein by volatilizing the menstruum therefrom.
4. In a process for the impregnation of wood, the step comprising immersing the wood in a liquid, non-aqueous menstruum comprising dimethyl ether, an impregnating agent being carried by the menstruum. 50
5. In a process for the impregnation of wood, the step comprising immersing the wood in a liquid, non-aqueous menstruum comprising dimethyl ether which contains dissolved carbon dioxide and a dissolved impregnating agent. 55
6. In a process for the impregnation of wood, the steps comprising treating the wood by injecting thereinto under pressure an impregnating agent dissolved in a liquid non-aqueous menstruum comprising dimethyl ether, and, after 60 impregnation of the wood, recovering the portion of the menstruum retained therein by volatilizing the menstruum therefrom.

7. In a process for the impregnation of wood, the steps comprising immersing the wood in a liquid, non-aqueous menstruum comprising dimethyl ether in which is dissolved an impregnating agent, sealing the wood and liquid menstruum in a closed receptacle, raising the temperature of the menstruum to obtain a corresponding pressure within the receptacle, withdrawing the liquid menstruum from the receptacle. 70

tacle, and volatilizing the portion of the menstruum retained in the wood to recover it therefrom.

8. In a process for the impregnation of wood,  
5 the steps comprising withdrawing air from the  
wood by preliminary vacuum, treating the wood  
under pressure with an impregnating agent dis-  
solved in a liquid, non-aqueous menstruum com-  
prising dimethyl ether, and, after impregnation  
10 of the wood, recovering the portion of the men-

struum retained therein by volatilizing the men-  
struum therefrom.

9. In a process for the impregnation of wood,  
5 the steps comprising impregnating the wood with  
zinc chloride dissolved in a liquid, non-aqueous  
menstruum comprising dimethyl ether, and, after  
impregnation of the wood, recovering the por-  
tion of the menstruum retained therein by vola-  
tilizing the menstruum therefrom.

ERNEST R. BOLLER. 10